

# UNITED STATES PATENT OFFICE.

HENRY ABBOTT, OF NEWARK, NEW JERSEY, ASSIGNOR OF THREE-FOURTHS  
TO WINTON C. GARRISON, OF SAME PLACE, AND THE ELGIN NATIONAL  
WATCH COMPANY, OF CHICAGO, ILLINOIS.

## PROCESS OF APPLYING COLORS TO ENAMEL DIALS FOR WATCHES AND CLOCKS.

SPECIFICATION forming part of Letters Patent No. 309,909, dated December 30, 1884.

Application filed March 10, 1883. (Specimens.)

*To all whom it may concern:*

Be it known that I, HENRY ABBOTT, of Newark, in the county of Essex, State of New Jersey, have invented certain new and useful  
5 Improvements in the Ornamenting of Enam-  
eled or Glazed Surfaces; and I do hereby de-  
clare that the following is a full, clear, and  
exact description thereof.

Heretofore colors have been applied to watch-  
10 dials and other enameled or glazed surfaces by  
hand with a brush or pencil, or by spreading  
the color over the surface to be ornamented,  
and after allowing said color to dry scraping  
away the surplus, so as to leave such only as  
15 formed the intended design. Each of the  
methods named is tedious and slow, and re-  
quires skilled, expensive labor, while the last-  
named method requires in addition the use  
of expensive and complicated machines espe-  
20 cially constructed for such purpose, and appli-  
cable to but a very limited range of designs.  
By another method impressions upon transfer  
paper have been taken from engraved plates  
and lithographic stones, and such impressions,  
25 while the color is soft, offset upon the surface to  
be ornamented; or by sticking the paper, with  
the impression upon its face, down upon said  
surface and allowing said paper to burn away  
when the article being ornamented is fired,  
30 leaving said colored design upon said article.  
The first of said last-named methods is liable  
to produce ragged or broken lines, or to spread  
the color if applied when too soft, and it is  
very difficult to place the design with accuracy  
35 upon the object to be ornamented, as the paper  
is not transparent and must be placed face  
downward, while by the second method the  
surface being decorated is liable to become  
stained or discolored by the burning paper.  
40 Certain photographic processes have also been  
devised for the purpose of placing colored  
designs upon glazed or enameled surfaces, but  
as they are uncertain in results, tedious, and  
expensive, they have not been used to any ex-  
tent.

The object of my invention is to place colored  
designs upon enameled or glazed surfaces with  
accuracy and rapidity and at a less expense  
than has heretofore been practicable; and to  
50 this end--

It consists, principally, in the method em-  
ployed for applying to and permanently se-  
curing upon enameled or glazed surfaces de-  
signs in vitrifiable colors, substantially as here-  
inafter specified.

It consists, further, in the method of pre-  
paring colored designs for the ornamentation  
of enameled or glazed surfaces, substantially  
as hereinafter shown.

It consists, further, in the method of remov-  
ing the transfer medium from a design during  
the operation of applying such design to and  
securing the same permanently upon a glazed  
or enameled surface, substantially as and for  
the purpose hereinafter shown.

It consists, further, in the method of pro-  
ducing transfer-films, substantially as and for  
the purpose hereinafter set forth.

It consists, finally, in the method of prepar-  
ing designs in color for transfer to enameled  
or glazed surfaces, substantially as and for the  
purpose hereinafter set forth.

To carry my invention into effect I first  
have the required design engraved or etched  
upon a metal or glass plate, preferably a cop-  
per plate. The colors ordinarily employed in  
encaustic painting on enamel are then rubbed  
into the engraved or etched lines in the same  
manner as for printing upon paper, after  
which I flow over the plate thus prepared a  
liquid collodion or other substance having  
similar properties, allow the collodion to set  
by evaporation, then place the plate thus  
coated in water, which may be made slightly  
acid, until the film becomes loosened from the  
surface of said plate, when it will either float  
to the surface of the water or may be readily  
stripped from the plate. As the collodion  
while in the liquid state will penetrate all the  
lines and recesses upon the surface of the plate,  
the coloring-matter will become embedded in  
or absorbed by it, and will come away from  
said plate with the film. The design engraved  
upon the plate thus transferred to the col-  
lodion film is not only upon the surface of said  
film, but is embedded in it, and if the opera-  
tion is carefully performed every particle of  
coloring-matter on the plate both in the finest  
and heaviest lines will be taken up. The col-  
lodion film may now be washed in clean water

55

65

75

85

95

100

and placed directly upon the enameled surface, either face down or reversed, and should be fastened in place by a thin varnish of gelatine—such as is used by photographers—or by a solution of sugar and water, or other colorless varnish, and then allowed to dry, after which the article being ornamented may be placed in the furnace and “fired” in the usual manner, the collodion quickly disappearing, being entirely consumed and leaving no trace, while the image or design is burned into the surface of the enamel in the same manner as if it had been applied by hand with a brush, or by any of the methods described. The 15 finest lines that can be engraved upon a plate will appear sharp and clear upon the enamel surface, while the heavy and deep cuts will be equally prominent. A single design, if accurately made on the plate, can thus be as accurately reproduced an indefinite number of times, and as many designs may be engraved on a single plate as can be conveniently handled, in which event after the film is stripped from the plate it may be cut into as many 25 pieces as required with a pair of shears. A convenient way to handle the film is to lay it upon a piece of wet paper and cut through both paper and film.

Two or more colors may be used in the same 30 transfer by rubbing the several colors in the parts of the plate where they are required, care being taken not to mix them.

The collodion used should be transparent and entirely free from coloring-matter, so that 35 the operator can see the design distinctly, and can place it accurately upon the enameled surface whether placed face down or reversed, and in order that no stains may be left upon the surface of the enamel after firing.

40 The collodion may be made in a variety of ways, but should be tougher than that ordinarily used by photographers. This is accomplished by using less alcohol and more ether and pyroxyline in the compound, which should be carefully filtered before using.

I find the following proportions to work satisfactorily: one ounce alcohol, four ounces ether, and one dram of pyroxyline. Gelatine and some other substances may also be 45 used for making the transfer, in the same manner as the collodion, but the latter is preferable. The transfer may also be made in the same manner from lithographic stones or photo-relief plates. When the liquid is flowed on the plate, the latter should either be placed 55 in a perfectly level position or made to revolve horizontally to insure an even distribution of the liquid over its surface. A single operator may manipulate a number of plates 60 at once by having the same arranged on a series of revolving stands operated by machinery.

After fixing the design upon the enameled surface with the varnish or glue and allowing 65 it to dry, the collodion film may be dissolved away by soaking in a solution of ether and alcohol, leaving the image or design adhering

to the varnish, after which other transfers in different colors may be added in the same manner as before; but in this case the film 70 must always be placed face down upon the enameled surface or the design will be carried away with the dissolving film. The best result can usually be obtained by dissolving away the film before firing, even in a single 75 transfer.

A striking advantage of my process over any heretofore employed for the same purpose is the fact that every detail of the original design is reproduced upon the enamel surface 80 very sharp and distinct.

Having thus fully set forth the nature and merits of my invention, what I claim as new is—

1. The method of placing figures or ornamental designs upon enameled or glazed surfaces, the same consisting in applying thereto a film of collodion or other similar material, having upon its surface and within its body the desired figures, numerals, or designs, and 90 causing said figures to adhere to and become a part of the enameled surface by the application of heat or otherwise, substantially as specified.

2. The method of applying to and permanently securing upon enameled dials and other 95 vitrified or vitrifiable surfaces designs in vitrifiable colors, consisting, first, in filling the sunk portions of a plate containing an engraved or etched design with the colored material, then flowing over said plate liquid collodion, and causing the same to permeate and become incorporated with said colored material, then removing from said plate the hardened film of collodion with its adhering and 100 incorporated design, then securing said film upon the surface of the article to be ornamented, and, lastly, subjecting said article to heat, whereby said vitrifiable colored material is fused and incorporated into the underlying 105 surface, substantially as shown.

3. The method of applying to and permanently securing upon enameled dials and other 110 vitrified or vitrifiable surfaces designs in vitrifiable colors, consisting, first, in filling the 115 sunk portions of a plate containing an engraved or etched design with the colored material, then flowing over said plate liquid collodion, and causing the same to permeate and become incorporated with said colored material, then removing from said plate the hardened film of collodion with its adhering and 120 incorporated design, then, by means of varnish or other adhesive substance, securing said film upon the surface of the article to be ornamented, and, lastly, subjecting said article to heat, whereby said vitrifiable colored material is fused and incorporated into the underlying 125 surface, substantially as set forth.

4. The method of preparing designs in colors 130 for ornamenting enameled, vitrified, or vitrifiable surfaces, which consists in causing said colors to adhere to and become incorporated with a film of collodion or other like

material, in substantially the manner and by the means herein described.

5. The method of applying to and permanently securing upon enameled dials or other vitrified or vitrifiable surfaces designs in vitrifiable colors, consisting, first, in securing upon the surface to be ornamented a film of collodion having upon or within the same the desired design in vitrifiable color, then re-  
10 moving the collodion by means of a solvent, leaving said design upon said surface, and, lastly, subjecting the article thus ornamented to the action of heat, whereby said vitrifiable color is fused and incorporated into the under-  
15 lying surface, substantially as specified.

6. The method of producing transfer-films, consisting, first, in filling the lines of an engraved or etched plate with colored material, then flowing over said plate liquid collodion  
20 and causing the same to permeate and become incorporated with said colored material, and, lastly, immersing said plate thus coated in acidulated water, whereby the film of col-

lodion with its adhering or incorporated design is loosened and may be separated, sub-  
25 stantially as shown.

7. The method of preparing transfer-films of collodion or other like material with figures or ornamental designs thereon, the same consisting in placing the colors on a plate of metal or other material having the characters, letters, designs, &c., engraved or etched thereon or therein, then flowing over the plate and over the colors contained on or within the engraved or etched portions of the 30 plate a film of collodion or other similar material, and then allowing or causing the collodion to harden by evaporation, whereby the letters, figures, &c., are caused to adhere to the collodion film, substantially as shown and 35 described.

HENRY ABBOTT.

Witnesses:

CHAS. F. EGLER, Jr.,  
CHAS. V. PEYU.